

## UNITED STATES PATENT OFFICE

JOHAN AXEL GUSTAFSSON, OF NORRTALJE, SWEDEN

## METHOD OF COATING SURFACES WITH A HARD COVERING

No Drawing. Application filed May 31, 1929, Serial No. 367,619, and in Sweden March 8, 1929.

- This invention relates to a method of coating surfaces with a hard covering which is weather-proof and resistive to injurious action and can be made in any colour desired.
- 5 The invention consists, chiefly, in coating the surface with a ground layer of glue insoluble in water, overstrewing with a mineral powder and, after drying, coating with filling mass, which consists of a drying oil and a 10 watery solution of an adhesive as well as a suitable quantity of a fine-grained mineral powder. After drying a very resistive, weather-proof covering is attained. Preferably, the surface is beforehand grounded with 15 such glue of thin consistency insoluble in water, said glue being left to dry completely before the other substances are applied. The filling mass mentioned above may also contain a pigment.
- 20 It is, of course, well known to use mineral matter in such coatings, but a characteristic feature of the present invention is the composition of the adhesives used to bind the mineral material.
- 25 In one preferred embodiment of the invention one or more layers of nitrocellulose or pyroxylin lacquer are applied on the surface, in combination with colour coatings for decoration, if desired.
- 30 When carrying out the method practically, for instance in treating a wooden surface, the surface is firstly primed or grounded with thin glue insoluble in water, preferably casein lime glue, which is left to dry, and then 35 a ground layer of such glue of a thicker consistency is applied and fine white sea sand (quartz sand) immediately sifted on. For certain purposes coarser sea sand, emery or glass powder or other mineral powder may be used 40 instead of the fine sea sand. If the sand is sifted on a horizontal surface the latter is afterwards raised to a vertical position thus causing all superfluous sand to fall off, so that a layer of suitable thickness uniformly 45 distributed over the whole surface will remain. The superfluous sand is gathered to be used again.
- When carrying out the method on a large scale in factories the glue is, preferably, applied by means of a suitable glue applying 50 machine, for instance having felt rollers, and the sand or powder is sifted on by means of a mechanically driven sifting device.
- This ground layer of sand and glue having dried thoroughly, an emulsion or filling mass 55 is applied, which is ground and mixed in a paint mill and consists of a drying oil, for instance boiled linseed oil, and a watery solution of paste, (preferably wheat flour paste), glue, casein, lime, gum, glair or the like together with a suitable quantity of fine-grained quartz powder and, if desired, a pigment. The watery solution of paste etc. on one hand and the drying oil on the other hand 60 are preferably used in equal parts in the emulsion, but the relative quantity of oil may also be less. It has been found, that also an emulsion containing paste and oil in the proportion of 2:1 may quite well be used. Instead of the quartz powder a fine-grained powder 65 of glass, emery, marble, gypsum, heavy-spar or other similar mineral material may be used. As a pigment zinc oxide or other light-proof and air-proof materials of the desired colour are used. A cheap and effective pigment is heavy-spar coloured with aniline colours.
- This emulsion or filling mass has the double purpose of filling out the space between the grains of sand in the underlying layer of 70 glue to give an even, smooth surface and of protecting against the action of moisture and temperature.
- When carrying out the method on a large scale in factories the filling mass is, preferably, applied by means of a machine having brush rollers.
- The coating thus attained which can be made in any colours desired and also be veined, marbled etc. in well-known manner, 75 can without any further treatment be used for many different purposes. If a further treatment of the surface is made or if the appearance is of no importance the pigment in the filling mass may be dispensed with.
- If a more decorative surface resistive to much moisture, lye, soap, spirits, ammonia etc. is necessary the surface produced in the manner described above is coated with one or 80 more layers of nitrocellulose or pyroxylin 85
- 100

lacquer. If the surface is to be decorated in a special manner, for instance by veining, marbling, decorative painting etc. such decoration is, preferably, made between two thin layers of coloured or colourless nitrocellulose lacquer. To vein and marble the usual pigments for such purposes may be used, such as terra sienna, van Dyke-brown, boneblack etc. For use the pigments are mixed either 10 with skimmed milk (casein solution) or in certain cases with a turpentine oil paint of low percentage of oil.

The coating of pyroxylin lacquer on the sand ground described becomes extremely 15 hard and resistive. The surface resembles a stone or a dressed brick wall surface and has a hardness approaching that of said materials. It has been found that pyroxylin lacquer on other ground does not by far give the 20 same good result. The pyroxylin lacquer is, preferably, sprayed on by means of an air brush or paint sprayer of usual design.

The method according to the invention 25 may advantageously be used for treating wood surfaces of all kinds as well as other surfaces, and is particularly adapted to make 30 plywood resistive to injurious action. The surfaces of the plywood sheets may for this purpose be treated in the factory so that only a treatment of the joints is necessary, when the sheets are set up.

The plywood sheet is coated on the front side as well as on the back side with glue and sand and with the filling mass and is thus 35 prevented from warping and completely protected against moisture. Moreover, the front side—and, if the sheet is to be set up in a place, where it will be exposed to very strong injurious action, also the back side—may be 40 treated with pyroxylin lacquer. The plywood sheet thus treated may, in spite of the great hardness of the coating, be bent to some extent without thus damaging the coating and may be worked by means of tools, for 45 instance be sawed, if a score is before cut through the hard coating down to the wood. To fasten the sheets with nails or screws a counter-sink for the nail or screw head is made in the hard coating.

50 On plywood or other sheets to be used for lining large surfaces on walls, ceilings or floors a margin about 1 cm. wide round the edges of the sheet is left without coating. After the sheets have been set up this margin 55 is treated in the same manner as the remaining portion of the surface, i. e. glue and sand are applied, filling mass is spread over, etc. In this manner also very large surfaces may be covered with plywood sheets and yet no 60 joints be visible. The joints may, however, be covered with laths having a coating according to the invention. Surfaces already set up, for instance, usual wooden walls may, of course, also be treated according to the 65 invention, though it is generally more advan-

tageous, from an economic point of view, to make the coating in the factory.

The method according to the invention 70 renders it possible to use wood for a plurality of purposes for which it has been less adapted heretofore, for instance, for linings for bathrooms and linings resistive to the action of weather for outside walls etc.

It is, of course, possible to use for the 75 water-proof glue another gluing substance which per se is soluble in water, such as animal glue, gelatine and the like and after its application treat it with a hardening substance, such as formaldehyde.

What I claim is:—

1. A method of coating surfaces with a hard covering, comprising coating the surface with a ground layer of glue insoluble in water, overstrewing with a mineral powder, and, after drying, applying a filling mass 85 consisting of a mixture of a drying oil, a watery solution of an adhesive and a fine-grained mineral powder.

2. A method of coating surfaces with a hard covering, comprising coating the surface with a ground layer of glue insoluble in water, overstrewing with a mineral powder, and, after drying, applying a filling mass 90 consisting of a mixture of a drying oil, a watery solution of an adhesive, a fine-grained mineral powder and a pigment.

3. A method of coating surfaces with a hard covering, comprising coating the surface with a ground layer of glue insoluble in water, overstrewing with a mineral powder, 100 after drying applying a filling mass consisting of a mixture of a drying oil, a watery solution of an adhesive and a fine-grained mineral powder, and, after drying, applying pyroxylin lacquer.

4. A method of coating surfaces with a hard covering, comprising coating the surface with a ground layer of glue insoluble in water, overstrewing with a mineral powder, 110 after drying applying a filling mass consisting of a mixture of a drying oil, a watery solution of an adhesive and a fine-grained mineral powder, and finally applying pyroxylin lacquer in several layers with intermediate layers of colouring substance.

5. A method of coating surfaces with a hard covering, comprising grounding the surface with thin glue insoluble in water, after 120 drying coating the surface with a ground layer of such glue of a thicker consistency, overstrewing with a mineral powder and, after drying, applying a filling mass consisting of a mixture, of a drying oil, a watery solution of an adhesive and a fine-grained mineral powder.

6. A method of coating surfaces with a hard covering, comprising coating the surface with a ground layer of glue insoluble in water, overstrewing with a mineral powder and, after drying, applying a filling mass 130

consisting of a drying oil and a watery solution of an adhesive in equal parts with an addition of a fine-grained mineral powder.

7. A method of coating surfaces with a hard covering, comprising grounding the surface with thin casein lime glue, after drying coating it with a ground layer of casein lime glue of a thicker consistency, overstrewing with fine quartz sand, after drying applying a filling mass, consisting of boiled linseed oil and a watery solution of glue in equal parts with an addition of fine-grained quartz sand, and finally applying pyroxylin lacquer in several layers with intermediate layers of colouring substance.

15 In testimony whereof I have signed my name.

JOHAN AXEL GUSTAFSSON.

20

25

30

35

40

45

50

55

60

65